

J. W. Smith,

Shoe Sole.

No 24,180.

Patented May 24, 1859.

Fig. 1.



Fig. 2.



Witnesses.

Platt, Verrett  
W. Croppfield

Inventor.

John W. Smith

# UNITED STATES PATENT OFFICE.

JOHN W. SMITH, OF WASHINGTON, DISTRICT OF COLUMBIA, ASSIGNOR TO HIMSELF, AND  
WALTER W. BERRY, OF BALTIMORE, MARYLAND.

## WATERPROOF SOLE.

Specification of Letters Patent No. 24,180, dated May 24, 1859.

*To all whom it may concern:*

Be it known that I, JOHN W. SMITH, of the city of Washington, in the District of Columbia, have invented a new and useful 5 Improvement in the Manufacture of Waterproof Inside Soles for Boots and Shoes; and I do hereby declare that the following is a full, clear, and exact description thereof, reference being had to the accompanying 10 drawings, making part of this specification, in which—

Figure I represents a plan view of the sole and Fig. II a vertical section.

My invention relates to improvements in 15 the manufacture of waterproof inside soles for boots or shoes whereby an important economical result is realized.

I prepare a composition of sixty-five parts by weight of coal tar, twenty parts of asphalt, ten parts of sulfuric acid of commerce, 20 and five parts of pulverized marble dust, whiting or gypsum, by thoroughly mixing the coal tar and asphalt, the former at boiling heat. When in a state of perfect solution a sample is set aside for the purpose of 25 ascertaining its consistency when cold. It should be of the consistence of vegetable tar at 60° F. If too thin add asphalt, if too thick add coal tar. When the mass is partly cooled add the sulfuric acid, a very little at 30 a time, stirring it in thoroughly all the time. If found to be too thick after adding the acid, it can be tempered by adding coal tar until it is sufficiently softened. When ready

to use the composition mix in pulverized 35 marble dust, whiting or plaster until the mass has done effervesing. This neutralizes the effect of the sulfuric acid upon the material upon which the compound is to be spread, which otherwise might be materially 40 injured. The acid destroys the offensive odor of the coal tar.

I make the soles by spreading a thin layer of the compound above described (a Fig. II) upon a sheet of coarse paper (b). 45 When it is hard, it is cut out in proper form by any convenient means, and canton flannel (c) is pasted on the side opposite to that on which the compound is placed and lapped over the edges. The sole is finished by pasting a piece of paper (d) over the composition to form the bottom of the sole.

I am aware that soles have been made of india rubber covered with cloth but such I do not claim. But, 50

What I do claim and desire to secure by Letters Patent as a new article of manufacture is—

The waterproof inside sole when constructed of the compound above described, 55 placed between two sheets of paper in the manner herein set forth.

In testimony whereof I have signed my name to this specification.

JOHN W. SMITH.

In the presence of—

CHAS. EVERETT,  
W. CROSSFIELD.